

## UNITED STATES PATENT OFFICE

GEORGE A. RICHTER, OF BERLIN, NEW HAMPSHIRE, ASSIGNOR TO BROWN COMPANY,  
OF BERLIN, NEW HAMPSHIRE, A CORPORATION OF MAINE

## PROCESS FOR THE PRODUCTION OF SULPHITE PULP

No Drawing. Original application filed November 1, 1926, Serial No. 145,708. Divided and this application filed July 20, 1928. Serial No. 294,319.

This invention relates to the production of chemical wood fiber by the sulphite process of digestion, and has for its object the production of a high grade sulphite pulp which is suitable for manufacture into bond, ledger and other writing paper of the highest quality, and which is an excellent raw material for the preparation of fiber of high alpha or resistant cellulose content.

10 For the production of sulphite pulp of high quality, it has been found preferable to digest wood chips in a liquor containing a soluble sodium salt, as, for example, in a sodium bisulphite solution having a combined  $\text{SO}_2$  content of about 2%, or greater, and a free  $\text{SO}_2$  content of about 5%. Such a liquor is particularly effective in penetrating the chips and in reacting with non-cellulosic constituents thereof, yielding an easily bleachable pulp having excellent paper making characteristics. The use of a sodium bisulphite solution as the digesting liquor, however, entails certain distinct disadvantages. Thus, in actual practice I have found that such liquor tends 25 to wear away the brick and cement lining of the usual sulphite digester, and that such lining is impaired far more rapidly and severely than when the usual calcium bisulphite liquor containing about 1% combined and 5% free  $\text{SO}_2$  and employed for the production of the usual commercial sulphite pulp, is employed. This disadvantage incident to the use of a solution of sodium bisulphite may be ascribed to the fact that, whereas a calcium bisulphite liquor assists in the preservation of the lining by depositing insoluble calcium salts, such as calcium sulphate and sulphite, in the form of a hard-baked scale on the lining during digestion, there is no tendency for such scale formation from a sodium bisulphite solution, because of the high solubility of the corresponding sodium salts. Consequently, instead of protecting the lining, a sodium bisulphite solution doubtless reacts with and dissolves 40 the lining material during digestion.

In accordance with the process of the present invention, I may employ as the fiber-liberating liquor a sulphurous acid solution of sodium bisulphite or other suitable soluble or 45 sodium salts containing suitable barium or strontium salts. Such a liquor makes possible the following advantageous features:

1. The production of an easily bleachable, high grade pulp.
2. The preservation of the digester lining, 55 owing to the decomposition of insoluble salts in the form of a protective coating on the lining.
3. The recovery of the valuable sodium constituent in the spent liquor of digestion, in a 60 condition suitable for reuse in the preparation of fresh cooking liquor.

When a process of fiber liberation such as hereinbefore described is practised in a plant equipped with a recovery system, one may employ a sodium bisulphite solution containing, say, about 2% combined  $\text{SO}_2$  and containing suitable barium or strontium salts, such as barium bisulphite, in sufficient amount so that when the digester is being relieved in 70 the final stages of cooking, the insoluble barium monosulphite is precipitated while free  $\text{SO}_2$  is escaping from the liquor. Barium sulphite and barium sulphate being of very low solubility, only a comparatively 75 very small amount of barium-bearing material need be added to the digested liquor to result in the precipitation of such salts during the final stages of digestion. Thus, about 10 to 30 pounds of barium carbonate need be added to the digester charge (depending on the size of the digester), the barium carbonate reacting with the sulphurous acid and forming barium bisulphite, which toward the end 80 of digestion is gradually precipitated as barium sulphite and sulphate, as free  $\text{SO}_2$  is released from the liquor.

The precipitation of barium monosulphite together with some sulphate gradually takes 85 place as the free sulphurous acid concentration of the cooling liquor is gradually decreased by the relief of free  $\text{SO}_2$  from the digester toward the end of the cook. Initially the liquor may be clear, as the high concentration of sulphurous acid increases the solubility of the monosulphite by reacting therewith to form the bisulphite which is more soluble than the monosulphite, but as the sulphurous acid which maintains the monosulphite in solution as bisulphite is decreased 90

95

100

in concentration, a precipitation of the more insoluble monosulphite takes place. For example, if the usual clear calcium bisulphite cooking liquor is boiled and the free  $\text{SO}_2$  liberated permitted to escape, a heavy precipitate of calcium monosulphite results. So, too, when a clear cooking liquor containing barium bisulphite is employed in a digester, as the liberation and escape of free  $\text{SO}_2$  proceeds, the more insoluble barium monosulphite is precipitated and deposits as scale on the digester lining.

The spent liquor resulting from digestion contains, however, but a small proportion of barium salts, so that it may be subjected to the evaporation and concentration steps without encountering excessive difficulty due to scale formation. Only a slight precipitate of barium sulphate and carbonate is produced in the smelt solution, so that filtration thereof is usually unnecessary. The smelt liquor may then be treated to produce a fresh sulphite liquor, sufficient suitable barium- and sodium-bearing materials being added to compensate for any losses in the cycle.

The barium-bearing material may be barium carbonate, barium hydroxide, or barium sulphate. Barium sulphate remains as such in the digesting liquor, only a relatively small proportion thereof being converted to barium bisulphite.

In lieu of barium bisulphite, strontium bisulphite may be used or formed in the sodium bisulphite solution in sufficient proportion to ensure toward the end of the cook the precipitation of strontium sulphite and sulphate which form as scale on the digester lining. Strontium sulphite is even more insoluble than barium sulphite so that in many cases it may be preferable to employ a sodium bisulphite solution containing strontium bisulphite as the cooking liquor. Strontium sulphate, however, is more soluble than barium sulphate, so that if only sulphate is the salt used in the cooking liquor, it is preferable to employ barium sulphate.

The advantageous features hereinbefore described may be realized when acid sulphite cooking liquors containing sodium salts other than sodium bisulphite are employed in the production of sulphite pulp, for instance a cooking liquor consisting of a sulphurous acid solution of sodium sulphite, as disclosed in my U. S. Patent No. 1,427,125, issued August 29, 1922. In such case, the pulping or fiber-liberating action is believed to be exercised by the small proportion of sodium bisulphite and sodium sulphite resulting from the reaction of the sodium sulphite with the free sulphurous acid, the larger proportion of sodium constituent remaining as sodium sulphate. Such a liquor contains a relatively high concentration of sodium constituent, and is preferably employed in a plant equipped with a recovery system. In accordance

with the process of the present invention, such a liquor may be treated approximately to saturation with certain barium or strontium salts. For example, certain basic barium salts, e.g., barium carbonate, may be added to the liquor, in which case barium sulphate is precipitated; or strontium carbonate may be added thereto, in which case strontium sulphite (which is more insoluble than strontium sulphate) is precipitated. Owing to the fact that barium sulphate has a much lower solubility than the other salts, it may be preferable to produce this particular salt in such liquor.

Inasmuch as certain barium and strontium salts may be successfully employed in carrying out the process of the present invention, I regard them as chemical equivalents. As there is no generic expression for both these salts (so far as I am aware), which does not include calcium salts, by the expression "barium" as used in the appended claims, I mean also to include strontium.

So far as subject matter is concerned, this is a division of my application Serial No. 145,708, filed November 1, 1926, which contains generic claims.

What I claim is:

1. A process which comprises digesting raw cellulosic material in a sulphurous acid solution of a soluble salt containing a barium salt in sufficient proportion therein to precipitate an insoluble barium salt when  $\text{SO}_2$  is released therefrom, and releasing  $\text{SO}_2$  from the solution during digestion to cause such precipitation.

2. A process which comprises digesting raw cellulosic material in a sulphurous acid solution of sodium salts containing barium salts.

3. A process which comprises digesting raw cellulosic material in a sulphurous acid solution of sodium salts substantially saturated with barium salts.

4. A process which comprises digesting raw cellulosic material in a sulphurous acid solution of sodium salts containing barium salts, concentrating the resulting spent liquor, and smelting and recovering the inorganic content of the concentrated spent liquor.

5. A process which comprises digesting raw cellulosic material in a sulphurous acid solution of sodium salts substantially saturated with barium salts, separating the resulting spent liquor, and smelting and recovering the inorganic content of the concentrated spent liquor.

6. A process which comprises digesting raw cellulosic material in a sulphurous acid solution of sodium bisulphite containing barium salts.

7. A process which comprises digesting raw cellulosic material in a sulphurous acid solution of sodium bisulphite containing barium bisulphite.

8. A process which comprises digesting

raw cellulosic material in a sulphurous acid solution of sodium bisulphite containing barium bisulphite in sufficient proportion to precipitate barium sulphite when  $\text{SO}_2$  is released therefrom.

5 9. A process which comprises digesting raw cellulosic material in a sulphurous acid solution of sodium bisulphite containing barium bisulphite in sufficient proportions to precipitate barium sulphite when  $\text{SO}_2$  is released therefrom, and releasing  $\text{SO}_2$  from the solution during digestion to cause such precipitation.

10 10. A process which comprises digesting raw cellulosic material in a sulphurous acid solution of a soluble salt containing a barium salt in sufficient proportion therein to precipitate an insoluble barium salt when  $\text{SO}_2$  is released therefrom, releasing  $\text{SO}_2$  from the solution during digestion to cause such precipitation, concentrating the resulting spent liquor, and smelting and recovering the inorganic content of the concentrated spent liquor.

15 11. A process which comprises digesting raw cellulosic material in a sulphurous acid solution of sodium salts containing a barium salt in sufficient proportion therein to precipitate an insoluble barium salt when  $\text{SO}_2$  is released therefrom, releasing  $\text{SO}_2$  from the solution during digestion to cause such precipitation, concentrating the resulting spent liquor, and smelting and recovering the inorganic content of the concentrated spent liquor.

20 12. A process which comprises digesting raw cellulosic material in a sulphurous acid solution of sodium bisulphite containing barium bisulphite in sufficient proportion to precipitate barium sulphite when  $\text{SO}_2$  is released therefrom, releasing  $\text{SO}_2$  from the solution during digestion to cause such precipitation, concentrating the resulting spent liquor, and smelting and recovering the inorganic content of the concentrated spent liquor.

25 13. A process which comprises digesting raw cellulosic material in a sulphurous acid solution of sodium bisulphite of about 2% combined  $\text{SO}_2$  content and containing barium bisulphite in sufficient proportion to precipitate barium sulphite when  $\text{SO}_2$  is released therefrom.

30 In testimony whereof I have affixed my signature.

GEORGE A. RICHTER.